

Jan. 14, 1947.

R. H. BROSEKER ET AL. 2,414,087  
METHOD OF PREPARING BAR STOCK IN THE MANUFACTURE OF  
PIEZOELECTRIC QUARTZ CRYSTALS  
Filed Aug. 10, 1942



Fig. 1



Fig. 2



Fig. 3



Fig. 4



Fig. 5

INVENTORS  
ROLAND H. BROSEKER  
BY JAMES L. HESSENAUER  
Joseph Q. Stanfield  
ATTORNEY

## UNITED STATES PATENT OFFICE

2,414,087

METHOD OF PREPARING BAR STOCK IN  
THE MANUFACTURE OF PIEZOELECTRIC  
QUARTZ CRYSTALS

Roland H. Broseker, Anne Arundel County, and  
James L. Hessenauer, Baltimore, Md., assignors  
to Bendix Aviation Corporation, South Bend,  
Ind., a corporation of Delaware

Application August 10, 1942, Serial No. 454,284

9 Claims. (Cl. 171—327)

**1**  
This invention relates to the preparation of bar stock in the manufacture of piezo-electric quartz crystals and more particularly to an optical method for determining the orientation of guide lines for the cutting of bar stock from a crystal slab.

In the past, the above determination has been made by employing a number of different pieces of test apparatus. Upon receiving the rough quartz crystals or aggregations of crystals, the position of the optical axis is determined either by well known optical methods or by the utilization of one of the undamaged faces of the crystal as a reference, if such a face exists. Because of the difficulty of making the determination optically, many establishments purchase only quartz crystals having at least one intact face and the entire crystal is cut up using this face as a reference. The cutting planes utilized are normally parallel to the basal plane and consequently are perpendicular to the optic or Z axis. The individual pieces thus obtained from each crystal are then kept together during the subsequent operations in order that the use of the reference face not be lost. Next, the slabs thus obtained are examined in polarized light to locate regions in which optical twinning is present and to determine the right-handedness or left-handedness of the crystal. For convenience in reference, the quality of right-handedness or left-handedness is sometimes termed the optical rotatory polarity. There are certain types of electrical twinning of the crystal which cannot be detected during these tests and as a result some pieces are not rejected until much further along in the process of fabrication after a considerable amount of work has been done on them. As the next step, the quartz is placed in a device for determining its polarity by means of the output voltage which is developed as a result of impact, and the crystal faces are marked accordingly. After obtaining this information, the slab is then cut up into rectangular bars using a cutting plane approximately normal to the first mentioned cutting plane. This plane may have any direction but usually lies along the Y or mechanical axis. The bar thus obtained is then inserted in a cutting machine and cut up into crystal blanks whose faces make the necessary angle with the Z axis to secure the desired temperature coefficient. For

**2**  
the type of cut known commercially as AT, this angle is approximately 35 degrees, 22 minutes, while the BT cut is made at an approximate angle of 49 degrees, 47 minutes. In the bar obtained as above, the Z axis is perpendicular to one of the sides, and the cuts, therefore, are made necessarily at a considerable angle to the major axis of the piece with the loss of much quartz.

It is an object of this invention to provide a method for the easy and rapid determination of guide lines for the cutting of bar stock in the manufacture of piezo-electric quartz crystals.

It is a further object of this invention to provide such a method which makes more efficient use of the crystal stock by eliminating waste inherent in previously known methods of determining guide lines and cutting bar stock from a crystal slab.

The above objects and advantages of the invention are accomplished by cutting crystalline quartz into slabs utilizing a cutting plane substantially parallel to the optical and mechanical axes, etching said slab in hydrofluoric acid, and passing a beam of light through said slab perpendicular to the optical axis. On the emergent face of the slab appear one or the other of two patterns of light which are indicative of the electrical polarity of the piece, which disclose whether it is right or left handed, and whose configurations indicate the lines along which bar stock must be cut to make the maximum number of crystal blanks having the required characteristic from a given piece of quartz.

Other objects and advantages will in part be obvious and in part be disclosed when the following specification is read in conjunction with the drawing in which:

Figure 1 illustrates a native crystal utilized in the preparation of piezo-electric resonators.

Figure 2 is a diagram showing the preparatory cut used on the native crystal.

Figure 3 is a section diagram illustrating the apparatus used in producing the desired images.

Figure 4 is an illustration of the pattern seen with a negative crystal face adjacent the observer in the apparatus of Figure 3.

Figure 5 is an illustration of the pattern seen with a positive crystal face adjacent the observer in the apparatus of Figure 3.

Figure 6 is an illustration showing the manner

in which the bar stock is cut out of the original crystalline slab of Figure 2.

Referring to Figure 1, there is shown such a crystal 1 of quartz or silicon dioxide as is more or less frequently encountered in nature. The optical axis 2 is located by using one of the crystal faces as a reference plane or by examining the crystal in convergent polarized light. The crystal 1 is now molded into a block of plaster of paris in such a manner that the optical axis 10 bears a predetermined relation to one of the surfaces of said block, this block serving as a jig to secure the crystal 1 while it is sawed into the slabs 3 of Figure 2 in a suitable machine. It will be noted from Figure 2 that the cutting planes are substantially parallel to the optical axis 2 and to the mechanical axis of the crystal. Upon the completion of the sawing operation, the slabs 3 are removed from the plaster of paris matrix and, when placed close together would have somewhat the form shown in Figure 2, whence the manner in which they were cut out of the crystal 1 is obvious. In preparation for the next step in the examination of the slabs 3, they are immersed in a suitable etching solution such as a 48% solution of commercial hydrofluoric acid for a period of three to four hours. At the completion of the etching process, they are removed from the solution and thoroughly washed and dried. The complete optical test set up is shown in Figure 3 in which 4 is an opaque rectangular enclosure secured to the top of the testing table 5 by the screws 6. Located within this enclosure 4 is a suitable light source such as the ordinary incandescent bulb 7 mounted in the socket 8. A pinhole 9 is pierced through the upper surface of the enclosure 4 directly above the light source 7. The specimen slab 3 to be tested is placed on the observation table formed by the upper surface of the enclosure where it is traversed by the light emanating from the pinhole 9, and the observer then inspects the patterns seen on the emergent surface of the slab 3, that is, the side nearest the observer, to determine the desired characteristics and the direction of cut for the preparation of bar stock from the slab. It will be noted that in this test, the Z axis is parallel to the surface of the testing table and the light from the pinhole therefore traverses the slab in a direction substantially perpendicular to that axis. A structure producing excellent results has been made by using .062 inch brass sheet for the enclosure 4 with a .013 inch circular opening for the pinhole 9.

The figures seen with the negative face of the crystal slab 3 adjacent the observer in the apparatus of Figure 3 are shown in Figure 4 in which the direction of the optical axis is indicated by the line 2. When a piece of left-handed quartz is examined, the solid line parallelogram 10 is seen, in which the short side is parallel to the optical axis and the long side makes an angle of approximately 52 degrees with this axis. The sides of this figure appear as bright lines against a gray or dark background. Since an AT cut crystal blank makes an angle of 35 degrees, 22 minutes with the optical axis, the long sides of the parallelogram may be used as guide lines for the cutting of bar stock from the slab 3 by merely placing a scale on the surface of the slab with its straight edge parallel to the desired side and scribing the necessary marks. A bar prepared in this manner is cut up into AT blanks by using a cutting plane inclined only 4 degrees to the minor axis of the bar rather than 35 degrees and

a considerable increase in the number of crystal blanks which may be obtained from a given piece of quartz is thereby effected due to the decrease in the amount of waste at the ends. A similar method may be used in the preparation of bars for the manufacture of BT cut crystal blanks. BT cut crystal blanks lie in a plane making an angle of 49 degrees, 47 minutes with the optical axis and the guide lines for the cutting of bar stock are therefore laid out substantially perpendicular to the long side of the parallelogram described above.

When a piece of right-handed quartz is examined, the dashed line parallelogram 11 of Figure 4 is seen and the AT bar stock in this case is again cut parallel to the long sides of the parallelogram. The manner in which the left-handed crystal is cut into bars is shown in Figure 6 in which the cutting planes 12 are clearly visible. With a positive face adjacent the observer, the double ended arrow 13 of Figure 5 is seen, the same image being present for both right and left-handed quartz. The arrow 13 lies perpendicular to the optical axis and along a mechanical axis of the crystal slab 3. In the present procedure, this arrow serves merely to identify the positive face although if desired it may be used as a reference to establish the cutting line.

When the above system is employed, it is no longer necessary to keep the groups of slabs cut from a native crystal of quartz together so that the reference plane is not lost, as the polarity, right-handedness or left-handedness, and the direction in which the cut is to be made are determined within a few seconds using the above method and apparatus. As the output of the slab cutting machines can thus be thrown into a common container and, after being etched, sent to the marking station and thence to the blank cutting station, mass production methods requiring little or no skill on the part of the operators can be employed. It has been found that the removal of the requirement for keeping individual slabs together has increased the output of the same group of personnel by a factor of three while the above method of cutting the bar stock has also appreciably increased the yield of crystal blanks from a given quantity of raw material.

There is a type of twinning termed electrical twinning which is not readily detected by optical methods. In a slab exhibiting this defect, the same figure is seen on both sides of the slab, that is, either the double ended arrow characteristic of the positive face or the parallelogram characteristic of the negative face. As would be expected, this type of quartz is inactive in that the piezo-electric effect is absent due to cancellation of the two polarities. This test is made by simply turning the slab over on the observation table and watching for the image change noted in good quartz. Very often slabs are found in which the polarity is not the same at all points and it is then desirable to lay out the lines of cut for the bar stock so that only one polarity exists within a given bar. Defects of this type are generally referred to as optical twinning. Using the apparatus of Figure 3, the lines of demarcation separating the regions of different polarity are readily located by simply sliding the slab about over the pinhole and watching the pattern changes whereby these lines may be readily sketched on the surface by the operator and the cutting planes for the bar stock laid out accordingly.

A few experiments have served to establish the fact that the character of the image observed is determined by the character of the emergent face which is remote from the pinhole. In one of these experiments a slab of quartz was prepared by polishing the positive face and etching the negative face. Placing this slab on the observation table of Figure 3 with the polished face adjacent the pinhole, the parallelogram characteristic of a negative face was seen by the observer. Upon the inversion of the piece, thus placing the negative face adjacent the pinhole, merely the pinhole itself was seen, the characteristic image being absent. However, as the piece was now lifted from the pinhole, the parallelogram indicating a negative face was once more seen, and this image increased in size as the separation between the pinhole and the negative face was increased. The parallelogram observed from the rear of the negative face had a slope which was the opposite of that in the figure observed from the front of the negative face. Thus, the pattern character is determined by the character of the face remote from the pinhole and its slope is dependent on the direction of light traverse.

While the cause for the existence of the above patterns is not precisely known, it is believed that they are produced by the action of regularly oriented crystalline facets on the light passing through them and that these facets are brought out from the structure of the slab by the action of the etching fluid. This hypothesis has been found to satisfactorily explain all the observed phenomena and appears to explain satisfactorily the fact that the images described above are destroyed if the etching process continues for too long a time. Since the action taking place is apparently in no way connected with the double refraction associated with crystalline quartz, this system of axis determination may also be employed in conjunction with other crystalline materials after preparation of the samples in a manner equivalent to that above described.

It will be obvious that many changes and modifications may be made in the invention without departing from the spirit thereof as expressed in the foregoing description and in the appended claims.

We claim:

1. In the manufacture of AT cut piezo-electric quartz crystals the method of preparing bar stock which comprises, cutting a slab from the mother crystal with a cutting plane substantially parallel to the Y and Z axes, etching said slab, placing said slab adjacent an illuminated pinhole with the positive face nearest the pinhole, marking said slab with a guide line substantially parallel to the long side of the parallelogram shaped light pattern seen in the negative face of said crystal slab, and cutting said slab along said guide line.

2. In the manufacture of AT-cut piezo-electric quartz crystals, the method of preparing bar stock which comprises, cutting a slab from the mother crystal with a cutting plane substantially parallel to the Y and Z axes, etching said slab, placing said slab adjacent an illuminated pinhole with the positive face nearest the pinhole, marking said slab with guide lines paralleling the long sides of the parallelogram shaped light pattern seen in the negative face of said slab within 15 degrees, and cutting said slab along said guide lines.

3. In the manufacture of BT-cut piezo-electric quartz crystals, the method of preparing bar

stock which comprises, cutting a slab from the mother crystal with a cutting plane parallel to the Y and Z axes, etching said slab, placing said slab adjacent an illuminated pinhole with the positive face nearest the pinhole, marking said slab with a guide line substantially perpendicular to the long sides of the parallelogram shaped light pattern seen in the negative face of said crystal slab, and cutting said slab along said guide line.

4. In the manufacture of BT-cut piezo-electric quartz crystals, the method of preparing bar stock which comprises, cutting a slab from the mother crystal with a cutting plane parallel to the Y and Z axes, etching said slab, placing said slab adjacent an illuminated pinhole with the positive face nearest the pinhole, marking said slab with guide lines perpendicular to the long sides of the parallelogram shaped light pattern seen in the negative face of said crystal slab within 15 degrees, and cutting said slab along said guide lines.

5. In the production of wafer like piezo-electric quartz crystal blanks, the method of manufacture which comprises, cutting a slab from the mother crystal with a cutting plane substantially parallel to the Y and Z axes, etching said slab, placing said slab adjacent an illuminated pinhole with the positive face nearest the pinhole, marking said slab with guide lines making an angle, which constitutes substantially an integral multiple of ninety degrees, with the long sides of the parallelogram shaped light pattern seen in the negative face of said crystal slab, cutting said slab into bars along said guide lines, and slicing said bars into wafers having their principal surfaces substantially perpendicular to said guide lines.

6. In the manufacture of AT cut piezo-electric quartz crystals the method of preparing crystal wafer blanks which comprises, cutting a slab from the mother crystal with a cutting plane substantially parallel to the Y and Z axes, etching said slab, placing said slab adjacent an illuminated pinhole with the positive face nearest the pinhole, marking said slab with guide lines substantially parallel to the long side of the parallelogram shaped light pattern seen in the negative face of said crystal slab, cutting said slab along said guide lines and cutting the resulting bars into wafers having their principal surfaces substantially perpendicular to said guide line.

7. In the manufacture of AT-cut piezo-electric quartz crystals, the method of preparing crystal wafer blanks which comprises, cutting a slab from the mother crystal with a cutting plane substantially parallel to the Y and Z axes, etching said slab, placing said slab adjacent an illuminated pinhole with the positive face nearest the pinhole, marking said slab with guide lines paralleling the long sides of the parallelogram shaped light pattern seen in the negative face of said slab within 15 degrees, cutting said slab along said guide lines, and cutting the resulting bars into wafers having their principal surfaces substantially perpendicular to said guide lines.

8. In the manufacture of piezo-electric quartz crystals, the method of preparing bar stock which comprises, cutting a slab from the mother crystal with a cutting plane parallel to the Y and Z axes, etching said slab, placing a cut face of said slab adjacent an illuminated pinhole, producing thereby a parallelogram shaped light dispersion pattern in the emergent face of said slab, and utilizing a side of said parallelogram as a reference for the marking of guide lines on said emergent face,

said guide lines making an angle with said long side which is substantially an integral multiple of ninety degrees.

9. In the manufacture of piezo-electric quartz crystals, the method of preparing bar stock which comprises, cutting a slab from the mother crystal with a cutting plane parallel to the Y and Z axes, etching said slab, placing a cut face of said slab adjacent an illuminated pinhole with the posi-

tive face nearest the pinhole, marking said slab with guide lines making an angle, which is substantially an integral multiple of ninety degrees, with the long sides of the parallelogram shaped light pattern seen in the negative face of said crystal slab, and cutting said slab along said guide lines.

ROLAND H. BROSEKER.  
JAMES L. HESSENAUER.